

[54] HIGH STRENGTH LOW COST STEEL FOR  
USE AT CRYOGENIC TEMPERATURES

[75] Inventor: John Joseph deBarbadillo, II,  
Warwick, N.Y.

[73] Assignee: The International Nickel Company,  
Inc., New York, N.Y.

[22] Filed: Jan. 31, 1972

[21] Appl. No.: 222,021

[52] U.S. Cl..... 75/123 K, 75/123 R, 148/36

[51] Int. Cl..... C22c 39/36, C22c 39/54

[58] Field of Search..... 75/123 R, 123 K; 148/36,  
148/134, 143

[56] References Cited

UNITED STATES PATENTS

3,619,302 11/1971 Aoki et al. .... 148/12  
2,258,604 10/1941 Gagnebin ..... 75/123 R

|           |         |                        |          |
|-----------|---------|------------------------|----------|
| 3,671,336 | 6/1972  | Korchynsky et al. .... | 148/36   |
| 2,204,585 | 6/1940  | Gagnebin ....          | 75/123 R |
| 2,451,469 | 10/1948 | Brophy et al. ....     | 75/123 R |
| 2,992,148 | 7/1961  | Yeo et al. ....        | 75/123 K |
| 3,388,988 | 6/1968  | Nagashimo et al. ....  | 148/36 X |
| 3,444,011 | 5/1969  | Nagashimo et al. ....  | 148/36 X |
| 3,620,717 | 11/1971 | Sekino et al. ....     | 75/123 K |
| 3,655,366 | 10/1969 | DePaul. ....           | 75/123 K |

OTHER PUBLICATIONS

Metallurgical Transactions, Vol. 1, December 1970,  
pgs. 3341-3350, Korchynsky et al.

Primary Examiner—Charles N. Lovel

[57] ABSTRACT

An alloy steel containing, among others, nickel, manganese, molybdenum, carbon and an element such as calcium, offers relatively high strength and excellent toughness at cryogenic temperatures.

2 Claims, 1 Drawing Figure



PATENTED MAY 21 1974

3,811,873



## HIGH STRENGTH LOW COST STEEL FOR USE AT CRYOGENIC TEMPERATURES

The subject invention is addressed primarily, but not exclusively, to the problem of producing an economical steel characterized by tensile strength and impact toughness of such magnitude as to render the steel suitable for use at cryogenic temperatures as low as -320°F., such properties being particularly useful in the production of storage vessels for liquified gases.

The processing and storage of liquified gases presents many problems, one of which is the selection of the most economical material of construction. At present, the so-called 8 percent and 9 percent nickel steels are being extensively used in these applications, with the specifications for these materials being set forth in ASTM Designation: A 553-70a. As is shown in the 9 percent nickel steel U.S. Pat. to Brophy and Miller, No. 2,451,469, cryogenic toughness is dependent on nickel content. This is demonstrated by comparing the 9 percent nickel steel, which is suitable for temperatures as low as -320°F., and the 8 percent nickel steel, which is limited to temperatures above -275°F. This temperature difference is significant since for many important industrial materials, such as LNG, tank fabricators require the steel to meet the specifications for temperatures as low as -320°F.

With the objective of developing lower cost materials for cryogenic applications, a variety of approaches have been advanced. One employs a unique heat treatment to 6-8 percent nickel steels, the treatment involving austenitizing, tempering above  $Ac_1$ , cooling, and then tempering at a temperature either above or below  $Ac_1$ . This approach is limited though, because of its inability to preserve the base plate properties in the weld-heat-affected zone, a property important in storage vessels where welding is, necessarily, extensively employed. Another approach involves modifying the alloying elements of the 6-8 percent nickel steels. This improves the properties to some extent but does not offer the level of properties, especially transverse toughness, capable of meeting the requirements imposed at temperatures below -275°F. Suffice to say, other proposals have been put forth, including strengthening the conventional 9 percent nickel steel such that thinner sections might be used. This too is not without objection.

In any case, it has now been discovered that satisfactory cryogenic properties may be brought together in one steel provided the steel contains correlated amounts of nickel, manganese, molybdenum, carbon, calcium, etc., as will be described more fully herein.

It is an object of this invention to provide a steel having a yield strength above about 85 ksi and an ultimate tensile strength above about 100 ksi together with Charpy V-notch toughness values of about 25, advantageously at least 30 ft.-lbs., or more in the longitudinal direction and about 20, preferably at least 25 ft.-lbs., or higher in the transverse direction at temperatures as low as -320°F.

Other objects and advantages will become apparent from the following description taken in conjunction with the accompanying drawing depicting a relationship between the percentages of nickel and manganese in the instant steel.

Generally speaking, the present invention is directed to a steel containing (by weight) from about 5 percent

to 7.5 percent nickel, from about 0.4 percent to 2.8 percent manganese, the manganese and nickel being correlated so as to represent a point within the area ACDEA of the accompanying drawing, from 0.01 to 0.5 percent molybdenum, the molybdenum and nickel being interrelated as set forth hereinafter, calcium in a small but effective amount to enhance toughness and up to about 0.1 percent, from about 0.05 to 0.14 percent carbon, up to about 0.5 percent silicon, up to about 0.1 percent columbium, the balance being essentially iron, the steel upon tempering, say at about 1,110° to 1,200°F., having a duplex microstructure comprised of a martensitic matrix containing dispersed austenite.

15 Nickel is essential in accordance herewith for strength and toughness since it acts as a stabilizer for the precipitated austenite dispersion. Amounts above 7.5 percent are unnecessary and a nickel range of 5.5 percent or 5.75 to 6.5 percent is highly satisfactory.

20 Manganese, as well as nickel, performs the role of lowering  $Ac_1$  so that an austenitic dispersion in a martensitic matrix is formed during tempering. In addition to this and in seeking an optimum combination of properties, notably transverse toughness, the percentages of 25 nickel and manganese should be correlated to represent a point in the area ACDEA of the accompanying drawing and advantageously within the area BCDEB. As will be shown hereinafter, the effect of manganese on the toughness properties, both longitudinal and transverse, is related to the nickel content. A manganese range of 1.75 to 2.5 percent together with 5.5 percent or 5.75 to 6.5 percent nickel affords good results.

30 The austenite dispersion is believed to be associated with or directly responsible for the outstanding cryogenic toughness in these nickel steels. Manganese, however, even at the low concentrations in these steels, to wit, 0.4-2.8 percent, has been found to be beneficial mostly, if not completely, in respect of longitudinal 35 toughness. Actually, it is deemed detrimental to transverse toughness, particularly in amounts of about 1 percent and higher, because it produces or contributes to a stringer-like inclusion morphology, the stringers seemingly being mostly sulfides. Transverse toughness can, as is well known, be brought to a level comparable to that in the longitudinal direction by employing more than the normal amount of cross rolling. This is expensive and thus unattractive (though full cross rolling is not excluded from the invention). Alternatively, high purity materials devoid of sulfur and other contaminants can be used as well as processing techniques designed to prevent or minimize the same. This too, also involves high cost and is thus not the most acceptable 40 panacea.

55 To negate this aforedescribed detrimental effect on transverse toughness it has been determined that certain elements alter the inclusion morphology from one of stringers or stringer-like to globular form. Calcium is particularly beneficial in this regard in amounts up to about 0.1 percent and in so doing contributes to bringing about an improvement in transverse properties. A retained calcium percentage of about 0.015 to 0.025 percent is quite beneficial, although a range of 0.005 percent or 0.01 to 0.05 percent is satisfactory. Other additives, such as magnesium, barium, strontium, zirconium and rare earths (particularly cerium), may also be 60 employed in similar amounts. As a consequence of this 65

aspect, the subject steel can contain even up to as high as 0.04 percent sulfur although lower levels, up to 0.015 or 0.02 percent, are preferred for weldability.

Molybdenum is used for toughness and solid solution strengthening. Additions of only 0.1 percent markedly enhance impact properties, both longitudinal and transverse, and increase strength. But it should be correlated to the nickel content, such that at 5 percent nickel it is at least 0.12 percent, at 5.5 percent nickel it is at least 0.08 percent, at 6 percent nickel it is at least 0.05 percent and at 7 percent nickel it is at least 0.01 percent. Above 7 percent nickel, molybdenum might be omitted but it is to be expected that properties would be lowered. (Interpolation can be used for intermediate percentages). Over the range of 5.5 to 6.5 percent nickel a molybdenum level of 0.08 to 0.15 percent is highly satisfactory.

Carbon has an important effect on toughness. Contrary to the general rule in these types of steels that toughness increases as carbon decreases, it was found that over the range of 0.05 to 0.13 percent or 0.14 percent there is a maximum level of toughness at approximately about 0.08 percent, i.e., about 0.07 to 0.09 percent. Toughness decreases gradually as the carbon content increases much above 0.08 percent but decreases rather sharply as it is lowered from 0.08 percent. To achieve the desired toughness, the carbon should be maintained advantageously above 0.05 percent, e.g., 0.06 percent or more, with the 0.08 percent level being most preferred. Although up to 0.2 percent might be tolerated, an upper limit of about 0.14 percent is beneficial since higher levels also contribute to welding problems.

In carrying the invention into practice, the steels can be produced in accordance with conventional procedures as those skilled in the art will appreciate. Both the melting steps and the casting and hot rolling steps may be carried out following conventional practices. The steel should be deoxidized with a material such as aluminum, e.g., up to 0.15 percent aluminum, according to fine grain practice. No unusual processing restrictions are required. As to heat treatment, it is preferred that the steels be austenitized for 1 hour at about 1,500°F., water quenched, and thereafter tempered for about 2 hours at about 1,125°-1,150°F. followed by a

water quench. The austenitizing temperature can be from 1,425° to 1,600°F. and the tempering temperature can be from 1,100° to 1,200°F. Air cooling can be used. Other heat treatments may be utilized such as the double normalize and temper (NNT) treatment employed in connection with the standard 9 percent nickel steel. The important consideration is tempering such that a two phase structure is achieved, to wit, a tempered martensitic matrix with a relatively fine and uniform dispersion of austenite, the austenite content being at least 3 percent, preferably at least 5 percent and most beneficially at least 10 percent by volume. The amount of austenite need not exceed 25 percent or 30 percent.

For the purpose of giving those skilled in the art a better understanding of the invention, the following description and illustrative data are given.

A number of steels were air-induction melted and cast into ingots. High purity raw materials were used. Electrolytic nickel and iron were used together with ferromanganese, ferrosilicon, etc. Deliberate additions of ferrophosphorus and ferrosulfide were made to simulate the purity in commercial 9 percent nickel steel. The charge was initially deoxidized with carbon and silicon-manganese. Final deoxidation was with aluminum. Calcium (calcium-silicon master alloy) was plunged into the melt after aluminum deoxidation. All the steels were unidirectionally rolled to  $\frac{1}{2}$  inch plate at 1,900°F. The steels were then given a uniform austenitizing treatment consisting of heating for one hour at 1,500°F., water quenching, tempering for 2 hours at 1,135°F. and again water quenching.

Smooth-bar tensile specimens were cut from the longitudinal direction of each heat treated plate. Charpy V-notch impact specimens were taken from both the longitudinal and transverse directions of the plates. The tensile tests were conducted at 70°F. and the impact tests were conducted at -320°F. Standard laboratory testing procedures were employed throughout this investigation.

The steels were of the following nominal composition (weight percent: 0.10 Mo, 0.25 Si, 0.12 C, 0.008 P, 0.015 S, 0.06 Al, 0.05 Cb and 0.015 Ca, the nickel and manganese contents being given in Table I together with tensile properties, including impact toughness, and the percentage of austenite.

TABLE I

| Alloy<br>No. | Ni<br>% | Mn<br>% | Austenite<br>Content,<br>% | Y.S.<br>ksi | U.T.S.<br>ksi | El.<br>% | CVN Impact<br>at 320°F. |        |
|--------------|---------|---------|----------------------------|-------------|---------------|----------|-------------------------|--------|
|              |         |         |                            |             |               |          | Long.                   | Trans. |
| 1            | 5.57    | 1.56    | 8                          | 107.6       | 120.9         | 25       | 28                      | 19     |
| 2            | 5.60    | 1.93    | 5                          | 119.8       | 128.1         | 20       | 27                      | 21     |
| 3            | 5.58    | 2.20    | 9                          | 114.5       | 126.3         | 21       | 28                      | 23     |
| 4            | 5.65    | 2.45    | 19                         | 109.6       | 128.7         | 25       | 29                      | 25     |
| 5            | 6.12    | 1.59    | 15                         | 98.8        | 127.7         | 27       | 31                      | 27     |
| 6            | 6.15    | 1.93    | 16                         | 103.7       | 128.9         | 25       | 33                      | 27     |
| 7            | 6.15    | 2.15    | 18                         | 112.2       | 129.3         | 26       | 30                      | 26     |
| 8            | 6.13    | 2.45    | 13                         | 120.5       | 132.3         | 23       | 28                      | 23     |
| 9            | 6.65    | 1.60    | 17                         | 103.6       | 126.7         | 27       | 35                      | 27     |
| 10           | 6.65    | 1.95    | 11                         | 120.0       | 131.3         | 22       | 33                      | 25     |
| 11           | 6.65    | 2.15    | 16                         | 118.6       | 131.5         | 22       | 34                      | 24     |
| 12           | 6.65    | 2.55    | 21                         | 116.6       | 133.8         | 24       | 30                      | 26     |

Y.S. = yield strength (0.2% offset)

U.T.S. = ultimate tensile strength

ksi = thousand pounds per square inch

El. = Elongation in 1 inch

Long. = Longitudinal

Trans. = Transverse

Table I reflects the desirability and advantage in correlating the nickel and manganese contents. At the lower nickel levels (e.g., Alloy 1), the manganese content should be maintained at the upper part of its range to achieve the desired transverse toughness (Alloys 3 or 4). Alloy 1 is at best a marginal steel and falls within the area ABEA of the drawing. In contrast, the more advantageous steels (Nos. 2-12) fall within the area defined by BCDEB. It might be added that at the higher nickel contents, toughness is not nearly as sensitive to changes in the manganese content, this being due to the overpowering effect of nickel in this regard. The nickel and manganese together with other austenite formers should be balanced against the ferrite formers. This can be accomplished by procedures well known to those skilled in the art (e.g., Schaeffler's diagram or modified versions thereof) so as to provide for a microstructure containing preferably at least 5 percent by volume of austenite.

Although the steels in Table I nominally contained 0.05 percent columbium, this constituent is not essential and it is preferred that it be omitted or at least be below 0.01 percent. A steel similar to Alloy 7 of Table I but to which columbium was not added exhibited a toughness level of 41 ft.-lbs. in the longitudinal direction and 38 ft.-lbs. in the transverse direction. This compares more than favorably with 30 and 26 ft.-lbs. respectively. Tensile strength was lower but not detrimentally so.

Carbon, as mentioned above and as can be seen from Table II, has the unexpected effect of producing a maximum toughness, both longitudinal and transverse, as the level is increased up to about 0.08 percent. The toughness decreases relatively rapidly at levels outside the range of about 0.07 to about 0.12 percent, particularly at the lower carbon levels. The alloys of Table II, apart from carbon, have the nominal composition (weight percent) of 6.1% Ni, 2.2% Mn, 0.1% Mo, 0.25% Si, 0.012% P, 0.016% S, 0.07% Cb and 0.015% Ca. It perhaps should be mentioned that, all other factors remaining the same, the impact strength of steels 13-16 would be expected to be higher if the steels were columbium-free.

TABLE II

| Alloy No. | C %   | Y.S. 0.2% Offset psi | Tensile Strength psi | Elong. % in 1 inch | CVN Impact at 320°F. |        |
|-----------|-------|----------------------|----------------------|--------------------|----------------------|--------|
|           |       |                      |                      |                    | Long.                | Trans. |
| 13        | 0.050 | 92,200               | 136,000              | 22                 | 21                   | 23     |
| 14        | 0.079 | 98,400               | 133,600              | 25                 | 39                   | 31     |
| 15        | 0.120 | 123,900              | 134,400              | 21                 | 32                   | 29     |
| 16        | 0.180 | 124,000              | 138,900              | 21                 | 25                   | 22     |

Table III shows the marked increase in transverse toughness caused by the addition of calcium or cerium. The steels, in addition to calcium or cerium, nominally contained 6.1% Ni, 2.1% Mn, 0.09% Mo, 0.2% Si, 0.13% C, 0.06% Cb, 0.006% P and 0.013% S.

verse directions, respectively, down to temperatures of about -320°F., and good weldability, said steel consisting essentially of from about 5.5 to about 6.5 percent nickel, manganese present in an amount up to about 2.8 percent, the nickel and manganese being correlated

TABLE III

| Alloy No. | Additive % | Y.S. 0.2% Offset psi | Tensile Strength psi | Elong. % in 1 inch | CVN Impact at 320°F. |        |
|-----------|------------|----------------------|----------------------|--------------------|----------------------|--------|
|           |            |                      |                      |                    | Long.                | Trans. |
| 17        | —          | 116,700              | 127,800              | 21                 | 35                   | 21     |
| 18        | 0.014 Ca   | 118,000              | 131,300              | 21                 | 36                   | 29     |
| 19        | 0.03 Ce    | 112,000              | 127,400              | 24                 | 36                   | 29     |

The alloys of the invention are weldable using such wires as the standard commercial wire used for 9 per-

cent nickel steel. Welding tests have shown that the weld metal and heat-affected zone have adequate toughness at -320°F.

The present invention contemplates articles, including structural elements, made from the nickel steels described herein, and subjected in use to load at temperatures as low as -320°F. Illustrative examples of such articles include tanks, containers, reservoirs, vessels, heat exchangers, and the like for producing, processing, storing and/or distributing liquified gas, and associated equipment such as valves, pumps, piping, tubes, conduits, structural shapes for reinforcing or restraining vessels, etc. The invention is particularly applicable for vessels containing such liquified gases as hydrocarbon gases, including natural gases, methane, propane, butane and other petroleum gases, and liquified nitrogen and liquified oxygen.

As will be understood by those skilled in the art, the use of the expression "balance" or "balance essentially" in referring to the iron content of the subject steel does not exclude the presence of other elements, such as those commonly present as incidental constituents, e.g., deoxidizing and cleansing elements, and impurities ordinarily associated therewith in small amounts which do not adversely affect the basic characteristic of the steel. Silicon in amounts up to about 0.5 percent, e.g., up to 0.3 percent, can be present. Phosphorus in normal amounts consistent with good steelmaking practice, for example, up to about 0.025 percent may also be present.

Although the present invention has been described in conjunction with preferred embodiments it is to be understood that modifications and variations may be resorted to without departing from the spirit and scope of the invention as those skilled in the art will readily understand. Such modifications and variations are considered to be within the purview and scope of the invention and appended claims.

I claim:

1. An alloy steel adapted for cryogenic applications and characterized by a yield strength above about 85,000 psi, Charpy V-notch toughness values of at least about 25 and 20 ft.-lbs. in the longitudinal and trans-

to represent a point within the area ACDEA of the accompanying drawing, at least 0.05 to 0.15 percent mo-

lybdenum, the nickel and molybdenum being related such that at the nickel percentages of 5.5 percent and 6 percent, the molybdenum is at least 0.08 percent and 0.05 percent, respectively, calcium present in an amount up to 0.1 percent to provide sulfide inclusions in globular form as opposed to the form of stringers, at least 0.06 percent and up to 0.14 percent carbon, and the balance essentially iron, said steel being further characterized by a duplex microstructure comprised of a martensitic matrix containing dispersed particles of austenite, the austenite being present in an amount of

at least 5 percent and up to about 25 percent by volume.

5 2. An alloy steel in accordance with claim 1 containing from 5.5 to 6.5 percent nickel from 1.75 to 2.5 percent manganese, from 0.05 to 0.12 percent molybdenum, about 0.01 to 0.05 percent calcium, at least 0.06 percent and up to 0.14 percent carbon, and the balance essentially iron, the austenite content being at least 10 percent.

\* \* \* \* \*

15

20

25

30

35

40

45

50

55

60

65

UNITED STATES PATENT OFFICE  
CERTIFICATE OF CORRECTION

Patent No. 3,811,873

Dated May 21, 1974

Inventor(s) JOHN JOSEPH deBARBADILLO, II

It is certified that error appears in the above-identified patent  
and that said Letters Patent are hereby corrected as shown below:

Col. 4, TABLE I, last column for "320°F." read -- -320°F. --.

Col. 5, TABLE II, last column for "320°F." read -- -320°F. --.

Col. 5, TABLE III, last column for "320°F." read -- -320°F. --.

Signed and sealed this 3rd day of December 1974.

(SEAL)

Attest:

McCOY M. GIBSON JR.  
Attesting Officer

C. MARSHALL DANN  
Commissioner of Patents